# EUROPEAN PATENT SPECIFICATION

(11) **EP 1 736 530 B1**
(45) Date of publication and mention of the grant of the patent: **03.02.2016**
(21) Application number: 05721627.7
(22) Date of filing: 29.03.2005
(51) Int. Cl.: C10M 169/04, C10M 105/04, C10M 137/02, C10M 137/10, C10M 159/24, C10N 20/00, C10N 20/02, C10N 30/00, C10N 30/06, C10N 10/04

(54) **LUBRICATING OIL COMPOSITION FOR CONTINUOUSLY VARIABLE TRANSMISSION**
SCHMIERÖLZUSAMMENSETZUNG FÜR KONTINUIERLICH VERÄNDERLICHES GETRIEBE
COMPOSITION D'HUILE LUBRIFIANTE POUR TRANSMISSION A VARIATION CONTINUE

(30) Priority: 29.03.2004 JP 2004097176
(43) Date of publication of application: 27.12.2006
(73) Proprietor: IDEMITSU KOSAN CO., LTD., Tokyo 100-8321 (JP)
(72) Inventor: HATA, Hitoshi, Ichihara-shi, Chiba 299-0107 (JP); KOGA, Hidetoshi, Ichihara-shi, Chiba 299-0107 (JP); MIYAJI, Tomomi, Ichihara-shi, Chiba 299-0107 (JP); TSUBOUCHI, Toshiyuki, Sodegaura-shi, Chiba 299-0293 (JP)
(74) Representative: Gille Hrabal
(86) International application number: PCT/JP2005/005886
(87) International publication number: WO 2005/093024

(56) References cited:
- EP-A- 0 989 177
- EP-A1- 0 968 987
- JP-A- 10 025 489
- JP-A- 11 349 969
- JP-A- 62 053 399
- JP-A- 2001 354 988
- JP-A- 2002 194 371
- JP-A- 2003 277 785
- JP-A- 2003 514 100
- US-B1- 6 320 088

## Description

### TECHNICAL FIELD

The present invention relates to the use of a lubricating oil composition in a metallic belt type continuously variable transmission or a chain type continuously variable transmission.

### BACKGROUND ART

There are known continuously variable transmissions (hereinafter occasionally referred to merely as "CVT") of various types, for example, a metallic belt type, a chain type and a traction drive type. Although any type of CVTs is required to have a high power transmission capacity, the power transmission performance of these CVTs varies depending upon properties of a lubricating oil used therein, more specifically, a metal-to-metal friction coefficient or a traction coefficient. The larger both coefficients are, the higher the power transmission capacity becomes.

The lubricating condition of the power-transmitting surface (a contact surface between metals) of the CVTs is considered to be a mixed lubricating condition including both an elastohydrodynamic lubrication (EHL) and a boundary/extreme pressure lubrication. In the metallic belt type CVT and the chain type CVT, the power-transmitting surface is mainly kept under the boundary/extreme pressure lubrication condition and, therefore, it is considered that the power-transmitting capacity thereof mainly depends upon the metal-to-metal friction coefficient. For this reason, as a base oil of the lubricating oil for CVTs of these types, there have been conventionally used hydrocarbon compounds such as paraffinic mineral oils and poly-α-olefins (PAO) to which additives are added to suitably control the metal-to-metal friction coefficient. On the other hand, in conventional traction drive type CVT, since the power transmission is performed through an EHL oil film, the power transmission capacity mainly depends upon the traction coefficient. Therefore, as a base oil of the lubricating oil for the traction drive type CVT, there have been conventionally used synthetic naphthenic compounds having a high traction coefficient. Thus, in CVTs of various type, special lubricating oils have been individually used (for example, refer to Japanese Patent Application Laid-open Nos. 09-100487 and 2001-288488).

However, in the metallic belt type CVT or the chain type CVT, the traction coefficient thereof is inherently small, and further the power transmission surface tends to undergo the change in shape of the friction surface when worn out by friction, thereby causing significant change in lubrication condition of the contact surface, etc. As a result, the metal-to-metal friction coefficient tends to be lowered, resulting in failure to accomplish desired power transmission and exhibit a good CVT function.

In addition, in the traction drive type CVT, the power transmission is partially performed in the boundary/extreme pressure lubrication manner under high-temperature and high-load conditions, so that the metal-to-metal friction coefficient at the contact surface tends to become unsatisfactory. As a result, the friction coefficient on the power-transmitting surface tends to be lowered, resulting in failure to attain desired power transmission, as well as less functional durability of the CVT.

For these reasons, it has been demanded to enhance a power transmission capacity of the respective types of CVTs, and improve a durability of CVT units by maintaining the enhanced power transmission capacity.
Further documents related to traction drive fluids are EP 0 968 987 A1, EP 0 989 177 A1, US 4,704,216 A, US 6,320,088 B1, US 6,372,696 B1, US 6,242,393 B1, US 2003/0181339 A1, JP 10-025489 A, JP 2001-354988 A and JP 2002-194371 A. According to the description of these documents, the use of the traction drive fluids is intended for conventional traction drive type CVT and none of these documents describes lubricating oil compositions for use in metallic belt CVT and chain type CVT.

### DISCLOSURE OF THE INVENTION

### PROBLEM TO BE SOLVED BY THE INVENTION

The present invention has been made in view of the above problems. An object of the present invention is to provide a lubricating oil composition for continuously variable transmission which is capable of enhancing a power transmission capacity of CVTs of a metallic belt type and a chain type, and maintaining the enhanced power transmission capacity.

### MEANS FOR SOLVING PROBLEM

The present inventors have found that when controlling a cohesive energy density of a base oil to a predetermined value or more, a metal-to-metal friction coefficient imparted by additives added thereto can be enhanced, and the enhanced friction coefficient can be maintained, and at the same time, such a base oil exhibits a high traction coefficient. The present invention has been accomplished on the basis of the finding.

Thus, the present invention provides:
[1] Use of a lubricating oil composition comprising:
   (A) a base oil comprising
      2-methyl-3-methyl-2-[(3-methylbicyclo[2.2.1]hepto-2-yl)methyl]bicyclo [2.2.1]heptane having a cohesive energy density at 40°C of 0.180 GPa or more,
      wherein said cohesive energy density (CED) at 40°C is calculated from the following formula (1): $CED \left(GPa\right) = 0.0204 \left(d/MW\right) ⋅ T ⋅ ln \left(2.51⁢η⋅MW\right)$
      wherein d is the density (g/cm³) at 40°C; MW is the molecular weight (g/mol);
      T is the absolute temperature (K); and η is the kinematic viscosity (mm²/s) at 40°C said base oil having a kinematic viscosity at 40°C of 5 to 150 mm²/s, and
   (B) a compound represented by the general formula (II):
   wherein r is 0 or 1; when r is 0, A is a hydroxyl group, and when r is 1, A is a hydrogen atom or a hydroxyl group; and R⁷ and R⁸ are respectively a hydrogen atom or a hydrocarbon group having 1 to 18 carbon atoms which may have one or more thioether bonds, and at least one of R⁷ and R⁸ is the hydrocarbon group having a thioether bond,
   in a metallic belt type and/or chain type continuously variable transmission.
[2] The use according to the above aspect [1], wherein said base oil (A) contains at least one compound selected from the group consisting of (i) dimerized norbornanes, (ii) hydrogenated dimers, trimers and tetramers of norbornanes and/or norbornenes, (iii) alkane derivatives having 2 or more cyclohexane rings, and (iv) alkane derivatives having one or more decalin rings and one or more cyclohexane rings.
[3] The use according to the above aspect [1] or [2], wherein the lubrication oil composition further comprises (D) a sulfur containing anti-wear agent.

### EFFECT OF THE INVENTION

The lubricating oil composition which is used according to the present invention is capable of enhancing a friction coefficient at a contact surface of a metallic belt type CVT and a chain type CVT, exhibiting an excellent wear resistance and, therefore, imparting a large power transmission capacity and a high durability to these CVTs.

### PREFERRED EMBODIMENTS FOR CARRYING OUT THE INVENTION

The base oil used as the component (A) in the present invention comprises the hydrocarbon compound 2-methyl-3-methyl-2-[(3-methylbicyclo-[2.2.1]hepto-2-yl)methyl]bicyclo[2.2.1]heptane having a cohesive energy density (hereinafter occasionally referred to merely as "CED") at 40°C of 0.180 GPa or more and preferably 0.200 GPa or more. When the CED at 40°C is 0.180 GPa or more, the base oil itself can exhibit a high traction coefficient, and further a composition obtained by blending the base oil with the component (B), etc., can exhibit a high metal-to-metal friction coefficient and at the same time, the effect of enhancing a wear resistance, so that the continuously variable transmission can be enhanced in power transmission capacity as well as persistency of the enhanced power transmission capacity.

The CED at 40°C is calculated according to the following formula (1):$CED \left(GPa\right) = 0.0204 \left(d/MW\right) ⋅ T ⋅ ln \left(2.51⁢η⋅MW\right)$
wherein d is the density (g/cm³) at 40°C; MW is the molecular weight (g/mol); T is the absolute temperature (K)i.e.T=303K; and η is the kinematic viscosity (mm²/s) at 40°C. Therefore, the CED at 40°C can be calculated by substituting the respective measured values for corresponding terms in the above formula (1).

Also, the base oil used as the component (A) in the present invention has a kinematic viscosity at 40°C of 5 to 150 mm²/s and preferably 8 to 50 mm²/s. When the kinematic viscosity at 40°C of the base oil is 5 mm²/s or more, the resultant composition can prevent wear of various mechanical elements of CVT or CVT units such as gears and bearings. When the kinematic viscosity at 40°C of the base oil is 150 mm²/s or less, the resultant composition is capable of preventing deterioration in low-temperature startability.

According to a preferred embodiment the base oil used as the component (A) in the present invention may contain a synthetic alicyclic hydrocarbon compounds selected from the following compounds (i) to (iv):
(i) dimerized norbornanes;
(ii) hydrogenated dimers, trimers and tetramers of norbornanes and/or norbornenes;
(iii) alkane derivatives having 2 or more cyclohexane rings; and
(iv) alkane derivatives having one or more decalin rings and one or more cyclohexane rings.

Examples of the above dimerized norbornanes (i) include those compounds represented by the general formula (I): wherein R¹ and R² are respectively a hydrogen atom or an alkyl group having 1 to 3 carbon atoms; R³ is a methylene, ethylene or trimethylene group which may have a methyl substituent group bonded to a side chain thereof n is 0 or 1; p and q are respectively an integer of 1 to 3 with the proviso that a sum of p and q (p + q) is an integer of 4 or less. These norbornanes are generally classified into two types according to the number n. That is, when n is 0, the general formula (I) is expressed by the following formula (I'): When n is 1, the general formula (I) is expressed by the following formula (I"):

Meanwhile, in the general formulae (I') and (I"), R¹ and R² are respectively a hydrogen atom or an alkyl group having 1 to 3 carbon atoms (such as methyl, ethyl, n-propyl and i-propyl); R³ is methylene, ethylene, trimethylene or these groups having a methyl group bonded to a side chain thereof (e.g., an ethylidene group and a methyl ethylene group); and p and q are respectively an integer of 1 to 3 with the proviso that a sum of p and q (p + q) is an integer of 4 or less.

These compounds represented by the general formulae (I') and (I") may be produced by various methods, and the production method therefore is not particularly limited. The compounds represented by the general formulae (I') and (I") may be usually produced by dimerizing norbornanes and/or norbornenes and then hydrogenating the resultant dimers.

The hydrogenated dimers, trimers and tetramers (ii) of norbornanes and/or norbornenes are hydrogenated products of dimers, trimers and tetramers (except for homopolymers of cyclic monoterpenoids) of either one or both of the norbornanes and norbornenes. As the norbornanes and norbornenes used herein as a raw material of the dimers, trimers or tetramers, there may be used various norbornanes and norbornenes without any particular limitations. Examples of the preferred norbornanes include those compounds represented by the following general formula: wherein R⁴, R⁵ and R⁶ are respectively a hydrogen atom or an alkyl group having 1 to 3 carbon atoms and preferably a hydrogen atom or methyl; and m is 1 or 2. Specific examples of the norbornanes include alkenyl norbornanes such as vinyl norbornane and isopropenyl norbornane; and alkylidene norbornanes such as methylene norbornane, ethylidene norbornane, isopropylidene norbornane, 3-methyl-2-methylene norbornane and 3,3-dimethyl-2-methylene norbornane. Examples of the preferred norbornenes includes those compounds represented by the following general formula: wherein R⁴ and R⁵ are the same as defined above; and k is 1 or 2. Specific examples of the norbornenes include, in addition to norbornene, alkyl norbornenes such as methyl norbornene, ethyl norbornene, isopropyl norbornene and dimethyl norbornene; alkenyl norbornenes such as vinyl norbornene and isopropenyl norbornene; and alkylidene norbornenes such as methylene norbornene, ethylidene norbornene and isopropylidene norbornene.

Specific examples of the alkane derivatives having 2 or more cyclohexane rings (iii) include 2,4-dicyclohexyl-2-methyl pentane and 2,4-dicyclohexyl pentane.

Specific examples of the alkane derivatives having one or more decalin rings and one or more cyclohexane rings (iv) include 1-cyclohexyl-1-decalyl ethane.

The above compounds all exhibit not only a high CED at 40°C but also, at the same time, a high traction coefficient. For example, the CED at 40°C and the traction coefficient at 100°C of some of the above-exemplified compounds are shown in Table 1 below.

Meanwhile, the CED is the value calculated from the above formula (1), and the traction coefficient is the value measured by the experimental method (experiment III) defined in the below-mentioned Examples.

**TABLE 1**

| Items | Base oil 1 | Base oil 2* | Base oil 3* | Base oil 4 | Base oil 5* | Base oil 6* |
|---|---|---|---|---|---|---|
| Kinematic viscosity at 40°C (mm²/g) | 21.8 | 19.9 | 12.2 | 18.4 | 34.3 | 28.2 |
| Density at 40°C (g/cm³) | 0.946 | 0.885 | 0.876 | 0.907 | 0.929 | 0.894 |
| Molecular weight (g/mol) | 246 | 250 | 236 | 277 | 248 | 287 |
| CED at 40°C (GPa) | 0.234 | 0.213 | 0.211 | 0.198 | 0.238 | 0.197 |
| Traction coefficient (100°C) | 0.1022 | 0.0973 | 0.0738 | 0.0679 | 0.098 | 0.0653 |

| | | | | | | |
|---|---|---|---|---|---|---|
| Note: Base oil 1: 2-methyl-3-methyl-2-[(3-methylbicyclo[2.2.1]hepto-2-yl)methyl]bicyclo[2.2.1]-heptane Base oil 2: 2,4-dicyclohexyl-2-methyl pentane Base oil 3: 2,4-dicyclohexyl pentane Base oil 4: Mixture of 75% by mass of the base oil 1 and 25% by mass of poly-α-olefin Base oil 5: 1-cyclohexyl-1-decalyl ethane Base oil 6: Mixture of 75% by mass of the base oil 5 and 25% by mass of poly-α-olefin *: not part of the invention | | | | | | |

As is apparent from Table 1, the CED and traction coefficient of the respective base oils have an correlation with each other, i.e., the higher the CED, the higher the traction coefficient becomes. When the CED at 40°C of the base oil is 0.180 GPa or more, the base oil itself exhibits a traction coefficient at 100°C of 0.06 or more.

The base oil as the component (A) may be composed of 2-methyl-3-methyl-2-[(3-methylbicyclo[2.2.1]hepto-2-yl)methyl]bicyclo[2.2.1]-heptane and the optional above synthetic alicyclic (cyclic saturated) hydrocarbon compound solely, or may be in the form of a mixture with a mineral oil or a chain hydrocarbon compound. Examples of the mineral oil include paraffinic mineral oils and naphthenic mineral oils. Examples of the chain hydrocarbon compound include poly-α-olefins.

The content of the mineral oil or chain hydrocarbon compound in the base oil is not particularly limited as long as the CED at 40°C of the base oil is 0.180 GPa or more, and is preferably in the range of 50% by volume or less on the basis of the base oil.

In the lubricating oil composition which is used for continuously variable transmission according to the present invention, the base oil as the component (A) is blended with the component (B) as explained below.

The component (B) used in the present invention is a phosphoric ester containing a hydrocarbon group having a thioether bond which is represented by the following general formula (II):

In the general formula (II), r is 0 or 1, and when r is 0, A is a hydroxyl group, whereas when r is 1, A is a hydrogen atom or a hydroxyl group. R⁷ and R⁸ are respectively a hydrogen atom or a hydrocarbon group having 1 to 18 carbon atoms which may have one or more thioether bonds. Examples of the hydrocarbon group having 1 to 18 carbon atoms include a linear or branched alkyl group having 1 to 18 carbon atoms, a cycloalkyl group having 3 to 18 carbon atoms, a linear or branched alkenyl group having 2 to 18 carbon atoms, an aryl group having 6 to 18 carbon atoms and an aralkyl group having 7 to 18 carbon atoms. Specific examples of the alkyl group having 1 to 18 carbon atoms include methyl, ethyl, n-propyl, isopropyl, n-butyl, isobutyl, sec-butyl, tert-butyl, pentyl, hexyl, octyl, 2-ethylhexyl, decyl, dodecyl, tetradecyl, hexadecyl and octadecyl. Examples of the cycloalkyl group having 3 to 18 carbon atoms include cyclopentyl, cyclohexyl, methyl cyclohexyl and cyclooctyl. Examples of the alkenyl group having 2 to 18 carbon atoms include allyl, propenyl, butenyl, octenyl, decenyl and oleyl. Examples of the aryl group having 6 to 18 carbon atoms include phenyl, tolyl, xylyl and naphthyl. Examples of the aralkyl group having 7 to 18 carbon atoms include benzyl, phenethyl and naphthylmethyl.

Examples of the hydrocarbon group having 1 to 18 carbon atoms which contains one or more thioether bonds include hexylthiomethyl, hexylthioethyl, octylthiomethyl, octylthioethyl, dodecylthiomethyl, dodecylthioethyl, hexadecylthiomethyl and hexadecylthioethyl. The R⁷ and R⁸ groups may be the same or different from each other, but at least one of the R⁷ and R⁸ groups is the hydrocarbon group having one or more thioether bonds.

Among the compounds represented by the general formula (II), examples of the acid phosphoric ester include those compounds having a structure represented by the general formula (II-a): wherein R⁷ and R⁸ are the same as defined above. Examples of the acid phosphoric ester represented by the general formula (II-a) include mono- or di-(hexylthioethyl)hydrogen phosphate, mono- or di-(octylthioethyl)hydrogen phosphate, mono- or .di-(dodecylthioethyl)hydrogen phosphate and mono- or di-(hexadecylthioethyl)hydrogen phosphate.

Also, among the compounds represented by the general formula (II), examples of the phosphorous ester include phosphorous esters having a structure represented by the general formula (II-b) or (II-c): wherein R⁷ and R⁸ are the same as defined above. Examples of the acid phosphorous ester represented by the general formula (II-b) or (II-c) include mono- or di-(hexylthioethyl)hydrogen phosphite, mono- or di-(octylthioethyl)hydrogen phosphite, mono- or di-(dodecylthioethyl)hydrogen phosphite and mono- or di-(hexadecylthioethyl)hydrogen phosphite.

In the present invention, the phosphoric esters containing a hydrocarbon group having a thioether bond as the component (B) may be used alone or in combination of any two or more thereof.

The component (B) serves for enhancing a wear resistance upon contact between metals and at the same time increasing a metal-to-metal friction coefficient, in the presence of the base oil as the component (A).

The amount of the component (B) blended in the composition of the present invention is 50 to 600 ppm by mass and preferably 100 to 400 ppm by mass in terms of the phosphorus content on the basis of the composition. When the amount of the component (B) blended lies within the range of 50 to 600 ppm by mass in terms of the phosphorus content, the resultant composition can ensure a good wear resistance and can be prevented from undergoing deterioration in oxidation stability.

The composition which is used according to the present invention may further contain an anti-wear agent as a component (D). The lubricating oil composition for CVT further containing the component (D) can be further improved in durability. Examples of the anti-wear agent include sulfides of animal and vegetable oils and synthetic oils such as sulfurized oils and fats, sulfurized olefins, polysulfides, sulfurized mineral oils, thiophosphoric acids, thiocarbamic acids, thioterpenes and dialkyl thiodipropionates. Specific examples of the sulfurized oils and fats include sulfurized lard, sulfurized rapeseed oils, sulfurized castor oils, sulfurized soybean oils, sulfurized rice bran oils, fatty acid disulfies such as oleic sulfide, and sulfurized esters such as sulfurized methyl oleate. Examples of the sulfurized olefins include those compounds obtained by reacting olefins having 3 to 20 carbon atoms or dimers, trimers and tetramers thereof, with a sulfurizing agent such as sulfur, sulfur chloride and other sulfur halides. Examples of the preferred olefins forming the sulfurized olefins include propylene, isobutene and diisobutene. The polysulfides are dihydrocarbyl polysulfides represented by the general formula (IV):

R¹⁰-Sₓ-R¹¹ (IV)

wherein R¹⁰ and R¹¹ are respectively an alkyl group having 1 to 20 carbon atoms, an aryl group having 6 to 20 carbon atoms, an alkylaryl group having 7 to 20 carbon atoms or an arylalkyl group having 7 to 20 carbon atoms, and may be the same or different from each other; x is a real number (more specifically, rational number) of 2 to 8.

Specific examples of R¹⁰ and R¹¹ in the general formula (IV) include methyl, ethyl, n-propyl, isopropyl, n-butyl, isobutyl, sec-butyl, t-butyl, various pentyl groups, various hexyl groups, various heptyl groups, various octyl groups, various nonyl groups, various decyl groups, various dodecyl groups, cyclohexyl, cyclooctyl, phenyl, naphthyl, tolyl, xylyl, benzyl and phenethyl. Examples of the preferred polysulfides include dibenzyl polysulfide, di-t-nonyl polysulfide and didodecyl polysulfide. Examples of the dithiophosphoric acids include zinc dialkyldithiophosphates and molybdenum dialkyldithiophosphates. Examples of the thiocarbamic acids include zinc dialkyldithiocarbamates and molybdenum dialkyldithiocarbamates. Examples of the thioterpenes include reaction products of phosphorus pentasulfide and pinene. Examples of the dialkylthiodipropionates include dilaurylthiodipropionate and distearylthiodipropionate. Among these sulfur containing anti-wear agents, preferred are sulfurized lard, zinc dialkyldithiophosphates, dilaurylthiodipropionates and isobutene sulfide, and more preferred are zinc dialkyldithiophosphates.

In the present invention, these sulfur containing anti-wear agents may be used alone or in combination of any two or more thereof. The content of the thiophosphates or the thiocarbamates as the sulfur containing anti-wear agent is preferably 0.2 to 2.0% by mass and more preferably 0.5 to 1.0% by mass on the basis of the composition. The content of the sulfur containing anti-wear agent other than the thiophosphates or the thiocarbamates is preferably 100 to 5000 ppm by mass and more preferably 400 to 3000 ppm by mass in terms of the sulfur content on the basis of the composition. When the content of the sulfur containing anti-wear agent lies within the above-specified range, the resultant composition can exhibit a good effect of improving an anti-seizing property and a wear resistance upon contact between metals.

The lubricating oil composition for CVT which is used according to the present invention can be obtained by blending the base oil as the component (A) with the component (B) mentioned above. The lubricating oil composition which is used according to the preferred embodiment of the present invention can exhibit a still higher total friction coefficient as well as a high wear resistance, so that a power transmission capacity of the continuously variable transmission can be more increased and the effect of keeping the high power transmission capacity can be attained.

The effect and mechanism of the present invention which can provide the above advantages are considered as follows. The friction coefficient observed on a power-transmitting surface of CVT is represented by the following formula (2): ${μ}_{total} = m ⋅ {μ}_{m} + \left(1-m\right) ⋅ {μ}_{t}$
wherein µₜₒₜₐₗ is a total friction coefficient; µₘ is a metal-to-metal friction coefficient; µₜ is a traction coefficient; and m is a ratio (Nₘ/N) of a load (Nₘ) supported by a contact portion between metals to whole load (N = Nₘ + Nₜ); and (1-m) is a ratio (Nₜ/N) of a load (Nₜ) supported by an oil film to the whole load.

Accordingly, if the load (pressing force) applied to the power-transmitting surface of CVT is kept constant and a sharing ratio of the load is kept constant, the total friction coefficient µₜₒₜₐₗ is influenced by the metal-to-metal friction coefficient µₘ at the surface and the traction coefficient µₜ of the EHL oil film.

The present inventors have found that the base oil having a high cohesive energy density (CED) exhibits a high traction coefficient, and has such an effect of enhancing the metal-to-metal friction coefficient µₘ and the wear resistance which are imparted by the component (B).

Therefore, by combining the base oil as the component (A) having a high traction coefficient µₜ with the components (B) having a high metal-to-metal friction coefficient µₘ enhanced by the component (A), the total friction coefficient µₜₒₜₐₗ can also be enhanced.

Further, when using the components (B) having the enhanced wear resistance, the power-transmitting surface can be inhibited from undergoing wear, so that the configuration of the power-transmitting surface such as surface roughness can be kept in an initial condition thereof. As a result, since the metal-to-metal friction coefficient, the traction coefficient and other factors remain unchanged, the total friction coefficient can be prevented from being deteriorated. For these reasons, it is suggested that the power transmission capacity is enhanced, and is inhibited from being lowered.

The lubricating oil composition for CVT which is used according to the present invention may further contain known additives unless the addition thereof adversely affects the objects of the present invention. Examples of the additives include detergent dispersants such as succinimide and boron-based succinimide; antioxidants such as phenol-based compounds and amine-based compounds; corrosion inhibitors such as benzotriazole-based compounds and thiazole-based compounds; rust preventives such as metal sulfonate-based compounds and succinic ester-based compounds; defoaming agents such as silicone-based compounds and fluorinated silicone-based compounds; and viscosity index improver such as polymethacrylate-based compounds and olefin copolymers. The content of the additives blended may be appropriately determined according to the objects and applications of the resultant composition. The total amount of the additives blended is usually 20% by mass or less on the basis of the composition.

### EXAMPLES

The present invention is described in more detail by referring to the following examples and comparative examples. However, it should be noted that these examples are only illustrative and not intended to limit the invention thereto. Meanwhile, various properties of the CVT lubricating oil were measured by the following methods.

### (1) Experiment I: Measurement of Friction Coefficient

A block-on-ring type friction test (LFW1 test) was conducted under the following friction conditions to measure a total friction coefficient after 5 min from initiation of the test at respective slide velocities.
Load: 1110 N (average Hertz stress upon initiation of the test: 0.49 GPa)
Oil temperature: 110°C
Test piece: Ring (φ35 x 5; SAE01 steel; RC60), Block (SAE4620 steel; RC60)
Slide velocity: 0.13 m/s, 0.25 m/s, 0.5 m/s and 1 m/s

### (2) Experiment II: Measurement of Friction Coefficient and Wear Resistance

A block-on-ring type friction test was conducted under the following friction conditions to measure total friction coefficients immediately after initiation of the test and after 60 min therefrom, and a width of wear on the block after the elapse of 60 min.
Load: 1530 N (average Hertz stress upon initiation of the test: 0.57 GPa)
Oil temperature: 130°C
Test piece: Ring (φ35 x 5; SAE01 steel; RC60), Block (SAE4620 steel; RC60)
Slide velocity: 0.37 m/s

### (3) Experiment III: Measurement of Traction Properties

The traction properties were measured by a twin-cylinder tester. A pair of metallic cylinders (material: bearing steel/SUJ-2; φ40/flat x φ40/r20; hardness: RC61; surface roughness Rm: 0.03) were disposed in an opposed relation to each other, and both rotated at 3300 rpm while applying a load of 147.1 N (average Hertz stress: 0.83 GPa) such that the difference in slide/roll ratio S.R. (=(U1 - U2) × 100/(U1 + U2) wherein U1 and U2 are velocities of the respective cylinders between both the cylinders) is 5%, to measure a tangential force F (traction force N) generated at a contact portion between the two cylinders, thereby determining a traction coefficient µₜ (= F/147.1).

### EXAMPLE 1 AND COMPARATIVE EXAMPLES 1 TO 3

Using base oils and additives shown in Table 2, the lubricating oil composition for CVT which is used according to the present invention (Example 1) and the comparative lubricating oil compositions for CVT (Comparative Examples 1 to 3) as shown in Table 3 were prepared to measure total friction coefficients thereof by the method described in the above Experiment I as well as traction coefficients thereof by the method described in the above Experiment III. The results of the measurement are shown in Table 3.

**TABLE 2-1**

| Base oil | Composition | CED at 40°C (GPa) |
|---|---|---|
| Base oil 1 | 2-methyl-3-methyl-2-[(3-methylbicyclo [2.2.1] hepto-2-yl)methyl]bicyclo[2.2.1]heptane | 0.234 |
| Base oil 2 | Naphthenic mineral oil (kinematic viscosity at 40°C: 27.9 mm²/s) | 0.178 |
| Base oil 3 | Paraffinic mineral oil (kinematic viscosity at 40°C: 20.3 mm²/s) | 0.128 |
| Base oil 4 | Poly-α-olefin (kinematic viscosity at 40°C: 30.0 mm²/s) | 0.101 |

**TABLE 2-2**

| Additive | Composition |
|---|---|
| Additive 1 | Di(octylthioethyl)hydrogen phosphite |
| Additive 2 | Boron-containing imide-based dispersant "ECA5026" available from Infineum Inc. (nitrogen content: 1.35% by mass; boron content: 0.35% by mass) |
| Additive 3 | Overbased calcium sulfonate "Bryton C400" available from Witoco Chemical Inc. (base value: 400 mg KOH/g; Ca content: 15.2% by mass; S content: 1.2% by mass) |
| Additive 4 | Reaction product of α-pinene and phosphorus pentasulfide "Hitec 649" available from Ethyl Japan Co., Ltd. (total acid value: 6.0 mg KOH/g; S content: 12.5% by mass; P content: 4.8% by mass) |

**TABLE 3**

| | Example | Comparative Examples | | |
|---|---|---|---|---|
| | 1 | 1 | 2 | 3 |
| Blending ratio (wt%) | | | | |
| Base oil 1 | 97.1 | | | |
| Base oil 2 | | 97.1 | | |
| Base oil 3 | | | 97.1 | |
| Base oil 4 | | | | 97.1 |
| Additive 1 | 0.4 | 0.4 | 0.4 | 0.4 |
| Additive 2 | 2.5 | 2.5 | 2.5 | 2.5 |
| Experimental results | | | | |
| Traction coefficient at 100°C | 0.0998 | 0.0552 | 0.0120 | 0.0050 |
| Total friction coefficient | | | | |
| Slide velocity: 0.13 m/s | 0.118 | 0.113 | 0.099 | 0.107 |
| Slide velocity: 0.25 m/s | 0.113 | 0.109 | 0.093 | 0.1 |
| Slide velocity: 0.5 m/s | 0.106 | 0.102 | 0.086 | 0.092 |
| /Slide velocity: 1.0 m/s | 0.102 | 0.096 | 0.076 | 0.082 |

### EXAMPLES 2 TO 4 AND COMPARATIVE EXAMPLES 4 TO 13

Using base oils and additives shown in Table 2, the lubricating oil compositions for CVT which are used according to the present invention (Examples 2 to 4) and the comparative lubricating oil compositions for CVT (Comparative Examples 4 to 13) as shown in Table 4 were prepared to measure total friction coefficients, wear widths and traction coefficients thereof by the methods described in the above Experiments I, II and III. The results of the measurement are shown in Table 4.

**TABLE 4-1**

| | Examples | | Comparative Examples | | |
|---|---|---|---|---|---|
| | 2 | 3 | 4 | 5 | 6 |
| Blending ratio (wt%) | | | | | |
| Base oil 1 | 99.6 | 97.1 | | | |
| Base oil 2 | | | 97.1 | | |
| Base oil 3 | | | | 97.1 | |
| Base oil 4 | | | | | 97.1 |
| Additive 1 | 0.4 | 0.4 | 0.4 | 0.4 | 0.4 |
| Additive 2 | | 2.5 | 2.5 | 2.5 | 2.5 |
| Additive 3 | | | | | |
| Additive 4 | | | | | |
| Experimental results | | | | | |
| Traction coefficient at 100°C | 0.1020 | 0.0998 | 0.0552 | 0.0120 | 0.0050 |
| Total friction coefficient | | | | | |
| Immediately after initiation of the test | 0.13 | 0.133 | 0.123 | 0.117 | 0.117 |
| After 60 min from initiation of the test | 0.114 | 0.118 | 0.112 | 0.108 | 0.107 |
| Wear width in block (mm) | 0.71 | 0.75 | 0.74 | 0.83 | 0.82 |

**TABLE 4-2**

| | Example 4 | Comparative Examples | | |
|---|---|---|---|---|
| | | 7 | 8 | 9 |
| Blending ratio (wt%) | | | | |
| Base oil 1 | 96.9 | | | |
| Base oil 2 | | 96.9 | | |
| Base oil 3 | | | 96.9 | |
| Base oil 4 | | | | 96.9 |
| Additive 1 | 0.4 | 0.4 | 0.4 | 0.4 |
| Additive 2 | 2.5 | 2.5 | 2.5 | 2.5 |
| Additive 3 | 0.2 | 0.2 | 0.2 | 0.2 |
| Additive 4 | | | | |
| Experimental results | | | | |
| Traction coefficient at 100°C | 0.0996 | 0.0550 | 0.0118 | 0.0050 |
| Total friction coefficient | | | | |
| Immediately after initiation of the test | 0.145 | 0.138 | 0.125 | 0.122 |
| After 60 min from initiation of the test | 0.128 | 0.12 | 0.116 | 0.114 |
| Wear width in block (mm) | 0.81 | 0.78 | 0.83 | 0.85 |

**TABLE 4-3**

| | Comparative Examples | | | |
|---|---|---|---|---|
| | 10 | 11 | 12 | 13 |
| Blending ratio (wt%) | | | | |
| Base oil SN3 | 99.5 | | | |
| Base oil MN1 | | 99.5 | | |
| Base oil MO2 | | | 99.5 | |
| Base oil SP3 | | | | 99.5 |
| Additive 1 | | | | |
| Additive 2 | | | | |
| Additive 3 | | | | |
| Additive 4 | 0.5 | 0.5 | 0.5 | 0.5 |
| Experimental results | | | | |
| Traction coefficient at 100°C | 0.1020 | 0.0555 | 0.0121 | 0.0050 |
| Total friction coefficient | | | | |
| Immediately after initiation of the test | 0.135 | 0.123 | 0.122 | 0.12 |
| After 60 min from initiation of the test | 0.098 | 0.093 | 0.09 | 0.084 |
| Wear width in block (mm) | 1.15 | 1.04 | 1.11 | 1.13 |

### INDUSTRIAL APPLICABILITY

The use of the lubricating oil composition for CVT according to the present invention as a general-purpose lubricating oil composition for metallic belt type CVT and chain type CVT increases the power transmission capacity thereof and enhances the durability thereof.

## Claims

1. Use of a lubricating oil composition comprising:
(A) a base oil comprising 2-methyl-3-methyl-2-[(3-methylbicyclo[2.2.1]hepto-2-yl)methyl]bicyclo [2.2.1]heptane having a cohesive energy density at 40°C of 0.180 GPa or more,
wherein said cohesive energy density (CED) at 40°C is calculated from the following formula (1): $CED \left(GPa\right) = 0.0204 \left(d/MW\right) ⋅ T ⋅ ln \left(2.51⁢η⋅MW\right)$
wherein d is the density (g/cm³) at 40°C; MW is the molecular weight (g/mol); T is the absolute temperature (K); and η is the kinematic viscosity (mm²/s) at 40°C said base oil having a kinematic viscosity at 40°C of 5 to 150 mm²/s, and
(B) a compound represented by the general formula (II): wherein r is 0 or 1; when r is 0, A is a hydroxyl group, and when r is 1, A is a hydrogen atom or a hydroxyl group; and R⁷ and R⁸ are respectively a hydrogen atom or a hydrocarbon group having 1 to 18 carbon atoms which may have one or more thioether bonds, and at least one of R⁷ and R⁸ is the hydrocarbon group having a thioether bond,
in a metallic belt type and/or chain type continuously variable transmission.

2. The use according to claim 1, wherein said base oil (A) contains at least one compound selected from the group consisting of (i) dimerized norbornanes, (ii) hydrogenated dimers, trimers and tetramers of norbornanes and/or norbornenes, (iii) alkane derivatives having 2 or more cyclohexane rings, and (iv) alkane derivatives having one or more decalin rings and one or more cyclohexane rings.

3. The use according to claim 1 or 2, wherein the lubrication oil composition further comprises (D) a sulfur containing anti-wear agent.

## Patentansprüche

1. Verwendung einer Schmieröl-Zusammensetzung, umfassend:
(A) ein Basisöl, umfassend 2-Methyl-3-methyl-2-[(3-methylbicyclo[2.2.1]hepto-2-yl)methyl]bicyclo[2.2.1]heptan mit einer kohäsiven Energiedichte bei 40°C von 0,180 GPa oder mehr,
wobei die kohäsive Energiedichte (CED) bei 40°C durch die folgende Formel (1) berechnet wird: $CED \left(GPa\right) = 0 , 0204 \left(d/MW\right) \cdot T \cdot ln \left(2,51 η\cdot MW\right)$
wobei d die Dichte (g/cm³) bei 40°C ist; MW das Molekulargewicht (g/Mol) ist; T die absolute Temperatur (K) ist; und η die kinematische Viskosität (mm²/s) bei 40°C ist, wobei das Basisöl eine kinematische Viskosität bei 40°C von 5 bis 150 mm²/s aufweist, und
(B) eine durch die folgende Formel (II) dargestellte Verbindung: wobei r 0 oder 1 ist; wenn r 0 ist, A eine Hydroxylgruppe ist und wenn r 1 ist, A ein Wasserstoffatom oder eine Hydroxylgruppe ist; und R⁷ und R⁸ jeweils ein Wasserstoffatom oder eine Kohlenwasserstoffgruppe mit 1 bis 18 Kohlenstoffatomen sind, die eine oder mehr Thioetherbindungen haben kann und mindestens einer von R⁷ und R⁸ eine Kohlenwasserstoffgruppe mit einer Thioetherbindung ist,
in einem stufenlosen Automatikgetriebe vom Metallriemen-Typ und/oder Kettentyp.

2. Verwendung nach Anspruch 1, wobei das Basisöl (A) mindestens eine Verbindung enthält, die ausgewählt wird aus der aus (i) dimerisierten Norbornanen, (ii) hydrierten Dimeren, Trimeren und Tetrameren von Norbornanen und/oder Norbornenen, (iii) Alkan-Derivaten mit 2 oder mehr Cyclohexanringen, und (iv) Alkan-Derivaten mit einem oder mehr Dekalinringen und einem oder mehr Cyclohexanringen bestehenden Gruppe.

3. Verwendung nach Anspruch 1 oder 2, wobei die Schmieröl-Zusammensetzung darüber hinaus (D) ein schwefelhaltiges Antiverschleißmittel enthält.

## Revendications

1. Utilisation d'une composition d'huile lubrifiante comprenant:
(A) une huile de base comprenant du 2-méthyl-3-méthyl-2-[(3-méthylbicyclo[2.2.1]hepto-2-yl)méthyl]bicyclo[2.2.1]heptane ayant une densité d'énergie cohésive à 40 °C de 0,180 GPa ou plus,
dans laquelle la densité d'énergie cohésive (CED) à 40 °C est calculée de la formule (1) suivante : $CED \left(GPa\right) = 0 , 0204 \left(d/MW\right) \cdot T \cdot ln \left(2,51 η\cdot MW\right)$
dans laquelle d est la densité (g/cm³) à 40 °C ; MW est le poids moléculaire (g/mol) ; T est la température absolue (K) ; et η est la viscosité cinématique (mm²/s) à 40 °C, ladite huile de base ayant une viscosité cinématique à 40 °C de 5 à 150 mm²/s et
(B) un composé représenté par la formule générale (II) : dans laquelle r est 0 ou 1; lorsque r est 0, A est un groupe hydroxyle et lorsque r est 1, A est un atome d'hydrogène ou un groupe hydroxyle ; et R⁷ et R⁸ sont respectivement un atome d'hydrogène ou un groupe d'hydrocarbure ayant de 1 à 18 atomes de carbone qui peut avoir un ou plusieurs liaisons de thioéther et au moins l'un de R⁷ et R⁸ est un groupe d'hydrocarbure ayant une liaison de thioéther,
dans une transmission à variation continue de type de courroie métallique et / ou de type de chaîne.

2. Utilisation selon la revendication 1, dans laquelle l'huile de base (A) contient au moins un composé sélectionné parmi le groupe consistant en (i) des norbornanes dimérisés, (ii) des dimères, trimères et tétramères hydrognénés des norbornanes et / ou norbornènes, (iii) des dérivés d'alkane ayant 2 ou plus cycles de cyclohexane et (iv) des dérivés d'alkane ayant un ou plus cycles de décaline et un ou plus cycle de cyclohexane.

3. Utilisation selon l'une des revendications 1 ou 2, dans laquelle la composition d'huile lubrifiante comprend en outre (D) un agent anti-usure contenant du souffre.
